

1

3,507,688

FLAMEPROOFED TEXTILE FABRICS AND  
METHOD THEREFOR

Wolfgang Carl and Martin Wandel, Dormagen, Dietrich Glabisch, Opladen, and Alfred Reichle, Dormagen, Germany, assignors to Farbenfabriken Bayer Aktiengesellschaft, Leverkusen, Germany, a corporation of Germany  
No Drawing. Filed June 5, 1967, Ser. No. 643,357  
Claims priority, application Germany, June 14, 1966,

F 49,460

Int. Cl. C09d 5/18

U.S. Cl. 117—136

6 Claims

## ABSTRACT OF THE DISCLOSURE

Flameproofed fabrics are prepared by applying to the fabric the reaction product of a polymer containing free anhydride groups, e.g. styrene-maleic anhydride copolymer, and a tri(halogenalkyl)-phosphate, e.g. tri(bromopropyl)-phosphate.

The present invention relates to flameproofed textile fabrics and a method for flameproofing textile fabrics and, in particular, floor coverings which comprise synthetic fibres only, by contacting them with a high molecular weight polymer containing phosphorus.

The use of a great many compounds for flameproofing synthetic moulded materials or synthetic fibres or filaments has already been proposed. For example, difficulty volatile organic bromine compounds and halogen-containing copolymers have been used for this purpose.

These known products do not, however, satisfy all the requirements which arise in connection with flameproofing of textiles. The use of flameproofing agents must not increase the attraction of the textile to dirt, and they must not be removable by vacuum cleaning, shampooing, or dry cleaning, and they must be resistant to abrasion. Furthermore, they must not affect detrimentally the physical properties of the filaments or fibres and in particular their mechanical strength.

It is an object of this invention to provide improved flameproofed textile fabrics, especially from synthetic fibres, used as floor covering and curtaining material, said flameproofed textile fabrics being treated with a reaction product of a polymer containing acid anhydride groups with a halogen-containing phosphoric acid ester.

A further object of this invention is a method for flameproofing textiles, in particular floor coverings and curtaining material which comprises treating the textile fabrics with a flameproofing agent consisting of a reaction product of polymers containing acid anhydride groups with halogen-containing phosphoric acid esters, as flameproofing agents and drying the treated textiles at temperatures from about 25° C. to about 130° C.

The phosphorus-containing and halogen-containing polymers which are used in the method according to the invention are prepared in known manner by reacting copolymers containing acid anhydride groups with phosphoric acid esters which contain halogen atoms. Copolymers which may be used include those obtained by copolymerisation of aryl-alkyl compounds which may also contain halogen, e.g. styrene,  $\alpha$ -methylstyrene,  $\alpha$ -methylstyrene,  $m$ -propylstyrene, 2,4-dimethylstyrene, ethylene, propylene, butylene, alkyl benzenes, with unsaturated acid anhydrides such as maleic acid anhydride or citraconic acid anhydride. The copolymers so formed may have a molecular weight of 10,000 to 80,000, preferably about 30,000. The halogenated phosphoric acid esters used are preferably tri(halogenalkyl)-phosphates, such as tri(chloroethyl)-phosphate, tri(dichloroethyl) - phosphate,

2

tri(trichloropropyl)-phosphate, tri(dichlorobutyl)-phosphate, tri(bromoethyl)-phosphate, tri(dibromoethyl)-phosphate or tri(dibromopropyl)-phosphate.

The reaction may be carried out in organic solvents or aqueous emulsions at elevated temperature, or by taking mixtures of the components in organic solvents or aqueous emulsions, evaporating off the solvents and reacting the undiluted products on the surface of shaped articles to form elastic films which are insoluble in water and organic solvents. Shaped textile materials, such as fibres of natural or synthetic origin, for example polyamide, polyacrylonitrile, polyester, cellulose and wool fibres and textile products manufactured from them, especially floor coverings and curtains, are rendered flameproof by the treatment with the high molecular weight phosphorus-containing polymeric reaction products. In general, the phosphorus and halogen-containing reaction products are applied from organic solvents or aqueous emulsions. The treated textiles have the additional advantage that they repel dirt to a greater extent than untreated textiles. Another advantage of the phosphorus- and halogen-containing reaction products is that after they have undergone complete reaction, the finish they produce is resistant to washing, cleaning, in particular using vacuum cleaners, shampooing and abrasion and vacuum cleaning, and in the case of floor coverings it is removed by constant wear by being walked over.

In contrast to known compounds that have flame inhibiting properties, the polymers used in the process according to the invention are particularly effective even when applied in small quantities. The polymers are most effective when used in quantities of only 3% to 15%, preferably 4% to 6%.

The following examples illustrate more particularly the invention.

## EXAMPLE 1

Tufted carpets of 80% polyacrylonitrile and 20% polyamide fibres (weight of pile about 1 kg./m.<sup>2</sup>) are sprayed with 300 ml./m.<sup>2</sup> of a solution which was prepared as follows:

100 g. of tri(2,3-dibromopropyl)-phosphate are dissolved in acetone together with 33.3 g. of a polymer of styrene and maleic acid anhydride of molecular weight about 30,000 and the solution is made up to 1 litre. The solution so obtained is then heated for 3 hours at 60° C. 6.7 g. of plasticiser, such as the monostearic acid ester of tri- $\beta$ -hydroxyethyl ammonium formate and 6.8 g. of an ethoxylated stearyl alcohol and 5 ml. of water are then added to the cooled solution with stirring.

After removal of the solvent by evaporation, and after drying for 24 hours at room temperature, a vacuum cleaner which has a beating action is passed over the carpet at a rate of 3 minutes per m.<sup>2</sup>. The carpet which has been spray treated undergoes change in neither colour nor handle. The percentage reduction in brightness of the treated carpet after soiling is found to be 22.7%. The corresponding value for untreated material is 22.4%. As a result of carrying out the flammability test according to DIN 51 960 (cellulose-ethanol test), the treated goods are classified as non-inflammable. The untreated carpet burns. When an attempt is made to ignite the carpet with a Bunsen burner, it is found that the carpet is difficult to ignite and is self-extinguishing.

## EXAMPLE 2

Tufted carpets of 100% polyacrylonitrile pile (weight of pile about 1 kg./m.<sup>2</sup>) are sprayed with 300 ml./m.<sup>2</sup> of an emulsion which was prepared as follows:

86.5 g. of tri-(2,3-dibromopropyl)-phosphate are added to 223 g. of a 12.9% solution in ethyl acetate of a polymer of styrene and maleic acid anhydride of molecular

weight about 20,000, this solution containing 28 g. of the polymer, and the solution is kept at boiling point for one hour. 5.7 g. of plasticiser, e.g. the monolauric acid ester of tri- $\beta$ -hydroxyethyl ammonium formate, 5.7 g. of an antistatic agent, e.g. a dodecylammonium compound, and 10 g. of emulsifier, e.g. benzyl hydroxydiphenylpolyglycol ether, are then added. 350 ml. of water are stirred into the solution by hand, a further 350 ml. of water is added. The mixture is then agitated with a high speed stirrer for one minute.

The sprayed carpets are dried in a drying cupboard at 80° C. for one hour, or at room temperature for 48 hours. A vacuum cleaner with a beating action is then passed over the carpet at the rate of 1 sq. m./min. The carpet is unchanged in colour and handle after this treatment. The percentage reduction in brightness of the sprayed carpet after soiling which is obtained is 24.1%. The reduction obtained for untreated goods is 23.8%. As a result of carrying out the flammability test, the treated carpet is classified according to DIN 51 960 (cellulose-ethanol test) as non-inflammable. Untreated goods burn. In the ignition test using a Bunsen burner both from the side and from above, the carpet is found to be inflammable only with difficulty and to be self-extinguishing.

#### EXAMPLE 3

Velour fabric made of polyacrylonitrile fibre is contacted in a padding machine adjusted to give 100% squeeze-out with an aqueous emulsion containing 84.4 grams/litre of the reaction product described below. The 30 velour fabric is then dried on a tentering frame at a temperature of 110° C. for a contact time of 1.5 minutes. The combustion period of the material, measured in an arc combustion testing apparatus, is then 105 seconds, and the flame extinguishes after a total combustion path 35 of 180°.

The emulsion used was prepared as follows:

173 g. of tri-(2,3-dibromopropyl)-phosphate are added to 223 g. of a 26% ethyl acetate solution of a polymer of styrene and citraconic acid anhydride of molecular 40 weight 15,000, which solution contains 59 g. of the polymer, and the reaction mixture is boiled for 1½ hours. 6.2 g. of plasticiser, e.g., the monostearic acid ester of tri- $\beta$ -hydroxyethylammonium formate, 5 g. of a dodecylammonium compound and 10 g. of emulsifier, e.g. o-benzyloxy-diphenylglycol ether, are then added. 358 ml. of H<sub>2</sub>O are stirred into the solution by hand, and, after the addition of a further 358 ml. H<sub>2</sub>O the solution is agitated using a high speed stirrer for 1 minute. The emulsion prepared in this way was then diluted to 3 litres with water 50 and was used for application in a padding machine.

#### EXAMPLE 4

Curtain fabric of polyacrylonitrile fibre is contacted in a padding machine adjusted to a squeezing effect of 100% with an aqueous emulsion which contains 100.5 grams/litre of the reaction product described below. The fabric is then dried on tentering frames at 110° C. for a contact time of 1.5 minutes. The combustion period of the material, tested in an arc combustion apparatus, is then 92 60

seconds and the extinction takes place at 90°. Untreated fabric burns over the total combustion path of 180°.

The emulsion used was prepared as follows:

213.6 g. of tri-(dichloropropyl)-phosphate are added to 223 g. of a solution in ethyl acetate of polystyrene 5 maleic acid anhydride of molecular weight 20,000, which solution contains 112 g. of the polymer. The solution is heated for one hour at 80° C. 9 g. of tri- $\beta$ -hydroxyethylammonium formate monododecyl ester is used as plasticiser, together with 5 g. of an antistatic, e.g. a dodecylammonium compound, and 10 g. of emulsifier, e.g. o-benzyloxy-diphenylpolyglycol ether, and 400 g. of water are then stirred by hand into the viscous solution. The solution is then made up to 1 litre with water and agitated using a high speed stirrer for one minute. 1 litre of the emulsion prepared in this way is diluted with water to 3 litres and used in the manner described above.

What we claim is:

1. Flameproof textile fabrics containing 3 to 18% by weight of the textile fabric of a flameproofing agent comprising:

(A) the reaction product of a copolymer having a molecular weight of 10,000 to 80,000 and containing acid anhydride groups, with

(B) an amount of tri-(halogenalkyl)-phosphate effecting to impart flameproof qualities to said textile.

2. Flameproof textile fabrics of claim 1, wherein said halogenated phosphoric acid ester is a tri-(halogenalkyl)-phosphate.

3. Flameproof textile fabrics of claim 1, wherein said copolymer is a copolymer of styrene and maleic acid anhydride having a molecular weight of about 20,000.

4. The flameproof textile fabrics of claim 1 wherein the weight ratio of copolymer and phosphate in the flameproofing agent is in the range of 1:3 to 3:1.

5. A method for flameproofing textile fabric comprising:

(1) applying to the fabric an organic solvent solution or an aqueous emulsion of a flameproofing agent comprising:

(A) the reaction product of a copolymer having a molecular weight of 10,000 to 80,000 and containing acid anhydride groups, with

(B) an effective amount of tri-(halogenalkyl)-phosphate; and

(2) drying the fabric; said flameproofing agent comprising 3 to 18% by weight of said fabric.

6. The method according to claim 5, wherein said treating is carried out with an emulsion of the reaction product.

#### References Cited

#### UNITED STATES PATENTS

2,660,543 11/1953 Walter et al. \_\_\_\_\_ 117—136

MURRAY KATZ, Primary Examiner

T. G. DAVIS, Assistant Examiner

117—138.8, 161 U.S. Cl. X.R.